

# UNITED STATES PATENT OFFICE.

JOHANNES HENDRIKUS PHILIPPUS LIGTERINK, OF Utrecht, NETHERLANDS.

## MANUFACTURE OF FLOOR-COVERING AS A SUBSTITUTE FOR LINOLEUM.

1,348,571.

Specification of Letters Patent.

Patented Aug. 3, 1920.

No Drawing.

Application filed November 23, 1918. Serial No. 263,922.

*To all whom it may concern:*

Be it known that I, JOHANNES HENDRIKUS PHILIPPUS LIGTERINK, expert, subject of the Queen of the Netherlands, residing at 5 Utrecht, Netherlands, 10.b Sweelinckstraat, have invented certain new and useful Improvements in the Manufacture of Floor-Coverings as a Substitute for Linoleum, of which the following is a specification.

10 The present invention relates to improvements in the manufacture of a floor covering as a substitute for linoleum.

In the British Patent No. 12,663, A. D. 1904, a method is described whereby a product is obtained, that is said to be a suitable article for substituting oilcloth or linoleum. Paper, treated with oil, water, size, soda and lime forms the foundation of that product. After drying, it is covered with a coat of oil, 15 and after that, if desired, the pattern which, owing to that coat of oil, does not become "dead", is put on to the upper side.

20 I have improved the above-said method in many respects.

25 I also start with paper as the body of the article, but in contradistinction to the paper in the above mentioned British Patent, the paper has through and through the fundamental color of the pattern to be put on, 30 which is done by applying the color in the "hollanders" to the paste board pulp. It must be understood, that the application of the color in the hollanders is already known.

35 Moreover the paper is made on the paper machine, in the thickness of ordinary linoleum, and in the quality of the so called "leather pasteboard" in rolls of unlimited length. It is already possible to make thin pasteboard in endless lengths (*papier sans fin*) by not passing the manufactured paper 40 through the cutting machines, which does not cause any difficulty, but was not done till now, as there was no need of it.

45 To make this leather pasteboard on the common paper machine, some modifications must be made to it. Firstly the paste board guide rolls must be of a larger diameter for preventing cracking the paste board. Besides, the wet-party (upon the copper gauze) 50 has to rise a good deal at the side of admission (side of the sluices) and accordingly it must be provided with a top sieve, to prevent flowing down of the milk, and to be sure of an equal thickness of the paste board.

Also the sieve itself must be sufficiently long 55 to effect proper drainage of the pulp, and the felt presses must be direct presses.

As a further improvement of the treatment according to the aforesaid British patent the paste board prepared in this way is 60 coated, front and back, with a mixture of equal parts boiled and unboiled linseed-oil. A double purpose is reached by it; in the first place the product becomes and remains extremely supple, because the unboiled linseed oil penetrates very far into the paper filaments, and in the second place the boiled linseed oil produces on the surface of the paste board a good base for putting afterward the coat of linseed oil color on it. In 65 the oilcloth technics the application of a mixture of boiled and unboiled linseed oil is already known.

70 After drying the paste board, treated in this way, front and back are painted with 75 linseed oil color, so as to make the product waterproof at both sides. The colors also being dried, the pattern is then put on one side; both last mentioned treatments as indicated in the aforesaid British patent.

75 In a word, the treatment is as follows: In the hollanders of a paper manufactory, the color that the paste board must become afterward as a fundamental color, is added to the pulp. This paste board is manufactured in the thickness of about  $\frac{1}{8}$ " (3 millimeters) on a paper machine, and this as endless paper, with a breadth of common linoleum. Accordingly it is the same color 80 through and through, and does not consist of layers pressed together, as is the case with common paste board obtainable up till now, and which is much too inflexible for the purpose desired.

85 The paste board manufactured in this manner is treated front and back with a mixture of equal parts boiled and unboiled linseed oil, and after drying repainted with a linseed oil paint in the color that the paste board already possessed. However 100 one side, that must become the wrong side, may be treated, if desired, with brownred linseed oil color, so as to obtain a product resembling common linoleum, which generally has that color on the wrong side.

105 After this coat of paint has dried sufficiently, the usual patterns are put on the right side in the wellknown manner.

Several of the above mentioned treatments are already known by themselves, although not all from the linoleum- or linoleum substitute industry. The invention 5 however consists of some connected under-treatments, which are partly known by themselves, but having as a result a new, practical, till now unknown article.

The advantages of it are, that it may be 10 manufactured and consequently obtained much cheaper than common linoleum, without being inferior to it in duration of life; besides, it is of a large insulating power to sound and heat, and in consequence of the 15 waterproof coat on both side, it can be used upon stone floors without fear of decay. The product being very elastic, seams of underlying wood floors will not soon mark themselves on the upper side of it. Finally, 20 the fundamental color of the pattern is always retained, although the design has

worn off, so that threadbare spots will not soon strike the eyes.

Having now fully described my said invention, what I claim and desire to secure 25 by Letters Patent is:

An improved method of manufacturing a floor covering as a substitute for linoleum consisting in adding a fundamental color for the finished product to the paper pulp, 30 in rolling the said paper pulp to the thickness of common linoleum, in treating the surfaces of said rolled product with liquid consisting of equal quantities of boiled and unboiled linseed oil, drying the same, coating both sides of said product with linseed oil, and applying a pattern to one surface 35 of the product.

In testimony whereof I have affixed my signature in presence of two witnesses.

JOHANNES HENDRIKUS PHILIPPUS LIGTERINK.